

(No Model.)

W. D. MARKS.  
METHOD OF MAGNETIZING.

No. 591,081.

Patented Oct. 5, 1897.



WITNESSES:

Horace A. Clark.

W. D. Marks

INVENTOR

William D. Marks

BY

Dyer & Driscoll  
ATTORNEYS

# UNITED STATES PATENT OFFICE.

WILLIAM D. MARKS, OF PHILADELPHIA, PENNSYLVANIA, ASSIGNOR TO THE AMERICAN ELECTRIC METER COMPANY, OF SAME PLACE.

## METHOD OF MAGNETIZING.

SPECIFICATION forming part of Letters Patent No. 591,081, dated October 5, 1897.

Application filed August 3, 1897. Serial No. 646,895. (No model.)

*To all whom it may concern:*

Be it known that I, WILLIAM D. MARKS, a citizen of the United States, residing at Philadelphia, in the county of Philadelphia, State 5 of Pennsylvania, have invented a certain new and useful Improvement in the Method of Magnetizing, of which the following is a specification.

My method of magnetizing consists in heating the steel to high heat—say up to red heat—by means of a melted-lead bath, Bunsen burners, or otherwise, and then immersing the steel in a water, mercury, or oil tempering-bath located between the poles of a strong electromagnet, thus simultaneously tempering and magnetizing the steel. By this method a molecular polarization of the steel is obtained while red-hot, and while in this condition and in the field of force of the magnet the steel is 15 tempered glass-hard. This avoids superficial magnetism and the consequent rapid deterioration of the permanent magnet or magnetic needle when put in use or laid aside.

The accompanying drawing illustrates a 20 form of apparatus which may be employed to carry my method into effect.

Referring to the drawing, A indicates a strong electromagnet whose cores *a* are provided with two pole-pieces *a'*. Between the 25 pole-pieces is supported a tank B, made of porcelain, zinc, rubber, or other suitable non-magnetic material. This tank contains a tempering-bath of water, mercury, oil, or other suitable fluid.

C represents the object to be treated, which 30 may be a piece of steel to be transformed into a permanent magnet or it may be a steel needle to be magnetized. The piece of steel will be held in proper position between the poles

of the magnet and in its field both while red- 40 hot and when plunged in the tempering-bath in an axial position.

A permanent magnet may be employed instead of the electromagnet if of sufficient strength. 45

What I claim is—

1. The method of tempering and magnetizing steel, consisting in first heating the steel to a sufficient degree then simultaneously subjecting the heated steel to the influence of a 50 magnet and immersing the heated steel in a tempering-bath, substantially as set forth.

2. The method of tempering and magnetizing steel, consisting in first heating the steel to a red heat and while red-hot subjecting the 55 steel to the influence of a magnet and immersing the steel in a tempering-bath while red-hot and in the field of force of the magnet, substantially as set forth.

3. In apparatus for tempering and magnetizing steel, the combination of a magnet and a tank made of non-magnetic material located between the poles of the magnet and containing a suitable tempering fluid, substantially 60 as set forth. 65

4. In apparatus for tempering and magnetizing steel, the combination of an electromagnet provided with pole-pieces, and a tank made of non-magnetic material located between the pole-pieces and containing a suitable tempering fluid, substantially as set forth. 70

This specification signed and witnessed this 30th day of July, 1897.

WM. D. MARKS.

Witnesses:

EDWARD P. HIPPLE,  
F. E. HIPPLE.